

## UNITED STATES PATENT OFFICE

1,965,710

## PHOTOMECHANICAL RESIST

Alexander Murray, Rochester, N. Y., assignor to  
Eastman Kodak Company, Rochester, N. Y., a  
corporation of New York

No Drawing. Application January 21, 1931,  
Serial No. 510,336

10 Claims. (Cl. 95—7)

This invention relates to a photo-mechanical resist or light sensitive enamel, such as is used in coating metal, light printing upon it from a halftone or line negative, developing, and then etching.

An object of the invention is the provision of a light sensitive enamel to replace the well known bichromated type of resist which has hitherto been used. As an example of the latter, fish glue and ammonium bichromate have been employed. Other colloids have also been used with bichromates. Another type of resist has consisted of certain light sensitive resins with sensitizers. Still another type is exemplified by Syrian asphaltum. In general, previous work in this field has depended upon the use of photo-sensitive organic materials in the colloidal or resinous state. As is well known, it is difficult to prepare compounds in this state of absolutely uniform composition and characteristics. Commonly, the composition is not even definitely known.

In the present invention, I use compounds of relatively high purity, which may generally be obtained in the crystalline state, and combine with them a substance or substances which inhibit or prevent the crystallization, make it possible to obtain a coating of a continuous film, and which cause the light sensitive compound to have a higher sensitivity than it would have in the crystalline state. The light sensitive compounds which are used are more or less well known for their property of light sensitivity, and many of the inhibitors which I add have been previously used in photo-mechanical resists.

The combination of these two types of substances is, however, new, and I produce from this combination a new result in that I prevent the light sensitive material from crystallizing and thereby obtain a continuous film of enhanced sensitivity having marked advantages.

The light sensitive substances which I use are complex unsaturated organic compounds of definitely known composition, in many cases it having been previously known that these materials are sensitive to light. These substances contain an ethylene linkage



Most of these substances show the property which is known as stereoisomerism, and under the action of light are converted from one isomer into another. As stated above, these properties have been previously described. For example, in 1895 C. Liebermann was so impressed by the sensitivity

of certain photo-polymerizations, notably the conversion of "allo-cinnamylidene-acetic acid"



60

into "trans-cinnamylidene acetic acid"



65

in benzol solution that he forecast a photographic use for the reaction. (Berichte 28, 1447.) In spite of this early prediction, however, very little practical use has been made of compounds of this type largely because of the very slight sensitivity of the materials when in crystalline state and their tendency to crystallize.

Compounds of the above-described class which give excellent results are the following: Anisal cinnamyl acetone, piperonylidene aceto-phenone, Cinnamylidene aceto-phenone, Benzylidene aceto-phenone, Iso (cis) cinnamal acetic acid.

These compounds are not directly applicable to the purpose of forming a continuous sensitive film. They crystallize when the volatile solvent evaporates, and in the crystalline state are only slowly affected by light.

I have found that if the substances can be maintained in a non-crystalline condition during exposure, they are much more sensitive to light. This and the means of doing it constitute in part the present invention.

A powerful inhibitor of crystallization is isonitroso acetophenone. One part of this to eight parts of anisal cinnamyl acetone, for example, is sufficient to prevent crystallization when the solvent evaporates. The film thus produced has some of the properties of a supersaturated solution. Copal resins are also inhibitors of crystallization, as are a number of other resins and gums. Some examples of gums and resins which I may employ are Cumar resin, pontiniak copal resin, and Kauri gum.

I do not limit myself by the examples given, as it is understood that other light sensitive substances and other gums and resins are useful.

While certain phases of the reaction which my sensitive layer undergoes are not perfectly understood, I believe that the first action of light on the light sensitive substance is to convert it from one isomer into another, and that on further exposure the second isomer is caused to polymerize. One possibility, in which two of

100

95

105

110

these isomers are polymerized to a dimer is shown by the following reaction:

5



10 The resins, gums, or other crystallization inhibitors employed are inert and indifferent substances, presumably taking no part in the reaction with light, and being apparently important only insofar as they affect physical characteristics of the film. It is believed that the non-crystalline film may be regarded as a solid solution, a fluid or plastic eutectic or a supercooled liquid. Whatever view may be taken as to the state of this film, it is only important, and a part of this invention, that the sensitive compounds are maintained in the non-crystalline state during exposure.

A general formula for practical use as a cold enamel in photo-mechanical work is:

Crystalline photo-sensitive compound..... 1.0 grams  
Non-sensitive inhibitor of crystallization..... 0.5 to 10.0 grams  
Acetone..... 15 c.c.

Most of the substances mentioned will give satisfactory results if used in accordance with this general formula.

Other specific formulas which give excellent results are the following:

*Example I*

|                                       |           |
|---------------------------------------|-----------|
| Anisal cinnamyl acetone.....          | 2.0 grams |
| Piperonylidine acetophenone.....      | 4.5 grams |
| Kauri copal XXX.....                  | 3.0 grams |
| Cumar resin, varnish grade, hard..... | 0.3 grams |
| Ethyl methyl ketone.....              | 25 c.c.   |
| Benzol.....                           | 25 c.c.   |
| Acetone.....                          | 50.0      |

Another formula is:

*Example II*

|                                  |           |
|----------------------------------|-----------|
| Piperonylidine acetophenone..... | 1.0 grams |
| Pontiniak copal.....             | 0.5 grams |
| Ethyl methyl ketone.....         | 5 c.c.    |
| Acetone.....                     | 10 c.c.   |
| Benzol.....                      | 5 c.c.    |

Another formula is:

*Example III*

|                        |           |
|------------------------|-----------|
| Michler's ketone*..... | 1.0 grams |
| Cinnamaldehyde.....    | 0.5 grams |
| Pontiniak copal.....   | 0.5 grams |
| Benzol.....            | 10 c.c.   |
| Alcohol.....           | 5 c.c.    |

\*tetra methyl diamino benzophenone

A formula which is cheaper is the following:

*Example IV*

|                                       | grams |
|---------------------------------------|-------|
| Anisal cinnamyl acetone.....          | 0.4   |
| Piperonylidine acetophenone.....      | 0.8   |
| Kauri gum.....                        | 1.0   |
| Cumar resin.....                      | 1.2   |
| Coumarin or m-nitro-benzaldehyde..... | 0.6   |

70 This formula is used as follows:

4 grams of the solids given above are dissolved in  
c.c.  
Acetone..... 30  
Benzol..... 10

In this formula the coumarin or m-nitro-benzaldehyde are used as a diluent and to make development easier.

Various substances may be used with the materials mentioned, as diluents or modifiers. These may be employed either to reduce the cost of the enamel, or to modify its characteristics. Such substances are for example, coumarin, m-nitro-benzaldehyde, p-nitroaniline,  $\beta$ -naphthol, p-nitro acetanilide, nitro-brom-benzene and p-nitro phenol.

80 85

A method of using these enamels is as follows: The metal, copper or zinc is scrubbed with pumice and water, rinsed, and the water polished off with a towel. Drying the water off on a whirler appears less satisfactory. After the metal plate is dry it is coated with one of the enamels given above, in an amber or orange light. The plate is then dried without heat in the dark for at least five minutes.

90 95

The plate is next exposed to an image, as under a suitable negative or by projection, to a strong light source, such as an arc, the exposure varying with the particular enamel used and usually lying between 15 seconds and 1 minute. To develop,

100 105

mineral oil is spread all over the print. This is kept in motion over the surface with absorbent cotton, being careful not to rub with too much force. Within one-half minute the unexposed part will become opaque and clearly visible. Development is continued for three minutes. Considerable pressure is now applied to the swab and the opaque areas come away. When all the opaque spots have been removed, the plate is then washed with soap and water and wiped dry. The 110 plate is now ready to etch and the known image areas will begin to etch instantly all over, when exposed to the etching fluid.

115 120

Advantages to be secured by the use of enamel made in accordance with this invention are as follows:

1. The enamel will stand any amount of treatment with nitric acid under 50% strength, and any amount of etching in ferric chloride.

2. It will stand the scrubbing of re-etching 120 brushes.

3. It will stand most water solutions, but not solvents, except paraffine and petroleum oils.

4. Because it is not brittle it does not "chew" at the edges in zinc etching, but etches with a 125 sharp even edge, giving perfectly formed dots in single-bite etchings.

5. It has a faint, pleasant aromatic odor, whereas many of the resists in use heretofore have a particularly strong and offensive odor.

130 135

In addition to these advantages, the sensitivity can be varied by adding more or less of the inactive substances or solvents. It is thus possible to obtain an enamel which prints within any time over a wide range.

Among substances which may be mentioned as modifiers are cellulose derivatives. Tackiness and solubility in the developer can be reduced by adding small proportions of cellulose ester solutions. As an example, 2 grams of 8% cellulose 140 nitrate in acetone are added to Example IV.

I consider as included within my invention all variations and equivalents coming within the scope of the appended claims.

145 150

What I claim is:

1. A photo-mechanical resist comprising, in a layer which is to be exposed to a light image, a crystallizable halogen-free organic light-sensitive substance capable of autogenic formation of insoluble chemically resistant non-crystalline prod-

ucts of higher melting point when exposed to light, together with a chemically indifferent substance which inhibits the crystallization of the light-sensitive material, so that said light-sensitive material is maintained in a non-crystallized state during exposure.

2. A light sensitive composition including in a non-crystalline state an unsaturated organic compound, light sensitive in itself, having the tendency to crystallize, and having the property when in non-crystalline state of isomerization under the influence of light and having such property to a very much less extent when in the crystalline state and a colloidal substance which inhibits the crystallization of the compound.

3. A composition for use as a photo-mechanical, light sensitive resist, including in solution an organic compound containing the ethylene linkage



said substance being light sensitive in itself, and having the property when in non-crystalline state of isomerization under the influence of light, and having such property to a very much less extent when in the crystalline state, and having a tendency to crystallize out of the solution, and a colloidal substance which inhibits the crystallization of the compound.

30 4. A light sensitive composition for use as a photo mechanical resist and including in solution a ketone containing the linkage



the ketone when in non-crystalline state being in itself light sensitive and when in crystalline state being light sensitive to a very much less extent, and a colloidal substance which inhibits crystallization of the ketone.

40 5. A light sensitive composition including in solution a ketone containing the linkage



the ketone when in non-crystalline state being in itself light sensitive and when in crystalline state being light sensitive to a very much less extent and a resin which inhibits the crystallization of the ketone.

50 6. A light sensitive composition including in solution an organic substance, capable when in non-crystalline state, when exposed to light, of auto-genic formation of insoluble chemically resistant non-crystalline products of higher melting point,

said substance having a tendency to crystallize and being substantially not light sensitive when in a crystalline condition, together with a colloid material which is inert with respect to the chemical or light sensitive properties of said substance, but which inhibits its crystallization.

5 7. A sensitive element comprising a support and a solid sensitive layer thereon, said layer comprising in a non-crystalline state an unsaturated organic compound, light sensitive in itself, having a tendency to crystallize, having when in non-crystalline state, the property of isomerization under the influence of light and having such property to a very much less extent when in crystalline condition and a colloid carrier which inhibits the crystallization of the compound.

8. A sensitive element comprising a support and a solid sensitive layer thereon, said layer including in a non-crystalline state an organic substance capable, only when in such state, of energetic autogenic formation of insoluble chemically resistant non-crystalline products of higher melting point, said substance having a tendency to crystallize, together with a colloid material which is inert with respect to the chemical and light sensitive properties of said substance but which inhibits its crystallization.

9. A sensitive element comprising a support and a solid sensitive layer thereon, said layer comprising in a non-crystalline state a ketone containing the linkage



said ketone being in itself appreciably light sensitive only when in a non-crystalline state and having a tendency to crystallize, together with a colloid material which is inert with regard to the chemical and light sensitive properties of said ketone but which inhibits its crystallization.

10. A sensitive element comprising a support and a solid sensitive layer thereon, said layer comprising in a non-crystalline state a ketone containing the linkage



the ketone being in itself appreciably light sensitive only when in a non-crystalline state and having a tendency to crystallize, together with a resin which is inert chemically and photo-genically toward the ketone but inhibits its crystallization.

ALEXANDER MURRAY.